# EUROPEAN PATENT SPECIFICATION

(11) **EP 2 358 930 B1**
(45) Date of publication and mention of the grant of the patent: **04.12.2013**
(21) Application number: 09796189.0
(22) Date of filing: 15.12.2009
(51) Int. Cl.: D01F 6/06, D01F 6/60, D01F 6/62, D01D 5/08, D01D 5/253

(54) **POLY-TRIMETHYLENE TEREPHTHALATE SOLID CORE FIBRILLATION-RESISTANT FILAMENT HAVING A SUBSTANTIALLY TRIANGULAR CROSS SECTION, A SPINNERET FOR PRODUCING THE FILAMENT, AND A CARPET MADE THEREFROM**
NICHTFIBRILLIERENDES MASSIVES ELEMENT MIT WEITGEHEND DREIECKIGEM QUERSCHNITT AUS POLYTRIMETHYLENTEREPHTHALAT, EINE SPINNDÜSE ZUR HERSTELLUNG DES ELEMENTS SOWIE EIN DARAUS HERGESTELLTER TEPPICH
FILAMENT RÉSISTANT À LA FIBRILLATION AVEC NOYAU SOLIDE DE TÉREPHTALATE POLYTRIMÉTHYLÈNE DE SECTION TRANSVERSALE SENSIBLEMENT TRIANGULAIRE, FILIÈRE DE PRODUCTION DU FILAMENT ET MOQUETTE RÉALISÉE À PARTIR DE CELUI-CI

(30) Priority: 18.12.2008 US 338412
(43) Date of publication of application: 24.08.2011
(73) Proprietor: E. I. du Pont de Nemours and Company, Wilmington, DE 19898 (US)
(72) Inventor: SAMUELSON, H., Vaughn, Chadds Ford Pennsylvania 19317 (US); SAMANT, K., Ranjan, Hockessin Delaware 19707 (US); CHANG, Jing, Chung, Boothwyn Pennsylvania 19061 (US)
(74) Representative: Hughes, Andrea Michelle
(86) International application number: PCT/US2009/067982
(87) International publication number: WO 2010/071775

(56) References cited:
- EP-A1- 1 219 732
- US-A- 5 176 926
- US-A- 5 686 121
- US-A- 6 048 615
- US-A1- 2005 266 241

## Description

### BACKGROUND OF THE INVENTION

This invention relates to a poly-trimethylene terephthalate solid core fibrillation-resistant synthetic filament, to a spinneret for producing the filament, and to a carpet made therefrom.

The ability of a tufted carpet made from synthetic polymeric filaments to retain its textured appearance, or "newness", tends to degrade over time. One cause of this appearance degradation is known as "fibrillation" that is produced by fraying of the carpet's filaments by use.

Various industry standard test methods, e.g., tetrapod walker test (ASTM D5251), hexapod walker test (ASTM D5252), Vetterman drum test (ASTM D5417), chair castor test and Phillips roll chair test are available to measure texture retention. Carpets samples are graded against a subjective scale after they have been subjected to these tests for predetermined number of cycles.

For example, tests performed on carpets made using petroleum-based poly-trimethylene terephthalate fibers having trilobal cross-section with a modification ratio of 2.0 and a 26.5 degree arm angle show significant fibrillation damage after 20,000 cycles in the Phillips roll chair test. Damaged trilobal filaments extracted from worn carpets after such test show severe deformities. One typical mode of deformation is manifested by adjacent lobes of the originally trilobal filament being bent toward each other, resulting in a filament having an elongated, compacted cross section. EP 1219732 A1 describes a polytrimethylene terephtalate fiber having a trilobal type modified cross-section.

In view of the foregoing it is desirable to produce filaments with cross-sections that are inherently more resistant to fibrillation, and are thereby able to provide superior texture retention during accelerated wear tests described above and exceptional durability in use. /

### SUMMARY OF THE INVENTION

The present invention is directed toward a solid core, fibrillation-resistant, synthetic polymeric filament having three substantially equal length convex sides. Each side meets an adjacent side through a substantially rounded tip centered on a respective circle of curvature spaced from the axis of the filament by a distance "a". Each rounded tip has a radius substantially equal to a length "b".

Each tip lies on a circumscribed circle having a radius substantially equal to a length (a + b) and the midpoint of each side lies on an inscribed circle having a radius substantially equal to a length "c". The filament having a modification ratio (MR) defined by the ratio of the radius (a + b) of the circumscribed circle to the radius (c) of the inscribed circle, wherein:
the filament has a denier-per-filament ("dpf") in the range 10 < "dpf" < 35;
the distance "a" lies in the range 0.00025 inches (6 micrometers) < "a" < .004 inches (102 micrometers);
the distance "b" lies in the range from 0.00008 inches (2 micrometers) < "b" < .001 inches (24 micrometers);
the distance "c" lies in the range from 0.0003 inches (8 micrometers) < "c" < .0025 inches (64 micrometers); and
the modification ratio ("MR") lies in the range from about 1.1 < "MR" < about 2.0.

More particularly,
the filament has a denier-per-filament ("dpf") in the range 12 < "dpf" < 32;
the distance "a" lies in the range 0.00035 inches (9 micrometers) < "a" < .003 inches (76 micrometers);
the distance "b" lies in the range from 0.00010 inches (3 micrometers) < "b" < .00095 inches (25 micrometers);
the distance "c" lies in the range from 0.0005 inches (10 micrometers)< "c" < .002 inches (51 micrometers); and
the modification ratio ("MR") lies in the range from about 1.1 < "MR" < about 2.0.

Preferably, the synthetic polymer is substantially poly-trimethylene terephthalate, and more preferably, the poly-trimethylene terephthalate has a 1,3 propane diol that is biologically produced. Alternately, poly-trimethylene terephthalate may come from renewably resourced routes. The synthetic polymer may be pigmented and/or may have a delusterant therein.

The filament has a tenacity greater than 1.5 grams per denier.

A carpet may be made from the filaments of the present invention.

The present,invention is also directed to a spinneret plate having a plurality of orifices formed therein for forming the solid core fibrillation-resistant, synthetic polymeric filament. Each orifice has a center and three sides with each side terminating in a first and a second end point and with a midpoint therebetween.

The first end point of one side is connected to the second end point of an adjacent side by a circular end contour having a radius equal to a dimension "C". The center point of each end contour is disposed a predetermined distance "D" from the center of the orifice.
The distance "C" lies in the range 0.0015 inches (38 micrometers) < "C" < .0040 inches (102 micrometers);
the distance "D" lies in the range from 0.0150 inches (381 micrometers) < "D" < .0300 inches (762 micrometers);
and more particularly:
the distance "C" may lie in the range 0.0020 inches (51 micrometers) < "C" < .0035 inches (89 micrometers);
the distance "D" may lie in the range from 0.0175 inches (445 micrometers) < "D" < .0280 inches (711 micrometers).

The present invention is also directed to a spinneret wherein the end contour connecting the first end point of one side to the second end point of an adjacent side is defined by at least two linear edges that intersect in an apex.

The first end point of each side is spaced from the second end point of an adjacent side by a baseline that itself intersects with a reference radius emanating from the center point. The intersection point between the baseline and the reference radius lies a distance "G" along the reference radius from the center of the orifice. The baseline has a predetermined length "2F". The apex is spaced a dimension "E" from an intersection of the baseline and the reference radius.
The distance "E" lies in the range 0.0025 inches (64 micrometers) < "E" < .0150 inches (381 micrometers);
the distance "F" lies in the range from 0.0015 inches (38 micrometers) < "F" < .0040 inches (102 micrometers); and
the distance "G" lies in the range from 0.0150 inches (381 micrometers) < "G" < .0300 inches (762 micrometers);
and more particularly:
the distance "E" may lie in the range 0.0030 inches (76 micrometers) < "E" < .0100 inches (254 micrometers);
the distances "F" may lie in the range from 0.0020 inches (51 micrometers) < "F" < .0035 inches (89 micrometers); and
the distance "G" may lie in the range from 0.0175 inches (445 micrometers) < "G" < .0280 inches (711 micrometers).

Regardless of the form taken by the end contour, each side of the orifice may be either substantially concave or substantially linear.

If orifice has substantially concave sides, each side lies on a reference circle having a radius of dimension "B". The center of the reference circle is located on a reference radius emanating from the center point of the orifice and passing through a midpoint of a side. The center of the reference circle is disposed a predetermined distance "A" along the reference radius from the central axis of the orifice.

The outermost point on each circular end contour lies on a circumscribed circle having a radius "(C+D)" (as defined above) centered on the center of the orifice. The midpoints of each side lying on a inscribed circle having a radius "H". [In the case of an orifice with concave sides the radius "H" is equal to the value (A-B)].

The orifice has a modification ratio ("MR") defined by the ratio of the radius (C+D) of the circumscribed circle to the radius "(A-B)" of the inscribed circle, thus,$" M ⁢ R " = \left(C+D\right) / " \left(A-B\right) " ,$
wherein
the distance "A" may lie in the range 0.0300 inches (762 micrometers) < "A" < .0900 inches (2286 micrometers);
the distance "B" may lie in the range from 0.0200 inches (508 micrometers) < "B" < .0800 inches (2032 micrometers);
the ratio (A/B) may lie within the range from about 1.0 < (A/B) < about 1.6; and
the modification ratio ("MR") may lie in the range from about 1.5 < "MR" < about 4.5.
More particularly:
the distance "A" may lie in the range 0.0300 inches (762 micrometers) < "A" < .0700 inches (2032 micrometers);
the distance "B" may lie in the range from 0.0200 inches (508 micrometers) < "B" < .0800 inches (1778 micrometers);
the ratio (A/B) may lie within the range from about 1.1 < (A/B) < about 1.5; and
the modification ratio ("MR") may lie in the range from about 1.8 < "MR" < about 3.5.

If an orifice has substantially linear sides with circular end contours the outermost point on each end contour again lies on a circumscribed circle having the radius "(C+D)" (as defined above) centered on the center of the orifice while the midpoints of each side lying on a inscribed circle having the radius "H" centered on the center of the orifice.

In the case of an orifice with linear sides and circular end contours the distance "H" (i.e., the radius of the inscribed circle) may lie in the range from:
0.0090 inches (229 micrometers) < "H" < 0.0190 inches (483 micrometers);
and more preferably, in the range from:
0.0108 inches (274 micrometers) < "H" < 0.0175 inches (445 micrometers).

The modification ratio ("MR") for such an orifice with substantially linear sides is also defined by the ratio of the radius (C+D) of the circumscribed circle to the radius "H" of the inscribed circle, thus,$" M ⁢ R " = \left(C+D\right) / " H " .$

The modification ratio ("MR") may lie in the range from about 1.6 < "MR" < about 2.5; and more particularly, the modification ratio ("MR") may lie in the range from about 1.7 < "MR" < about 2.3.

For orifices having linear sides and linear end contours the distance "H" (i.e., the radius of the inscribed circle) may lie in the range from:
0.0088 inches (224 micrometers) < "H" < 0.0185 inches (470 micrometers)
and more preferably, in the range from:
0.0105 inches (267 micrometers) < "H" < 0.0170 inches (432 micrometers) .

The modification ratio ("MR") for orifices having linear sides and linear end contours is also defined by the ratio of the radius (E+G) of the circumscribed circle to the. radius "H" of the inscribed circle, thus,$" M ⁢ R " = \left(E+G\right) / " H "$

The modification ratio ("MR") may lie in the range from about 1.6 < "MR" < about 2.5, and more particularly, the modification ratio ("MR") may lie in the range from about 1.7 < "MR" < about 2.3.

### BRIEF DESCRIPTION OF THE DRAWINGS

The invention will be more fully understood from the following detailed description taken in connection with the accompanying Figures, which form a part of this application and in which:
Figure 1 is an end view of a filament in accordance with the present invention taken in a plane perpendicular to the longitudinal axis of the filament;
Figure 2A is an end view a first embodiment of a spinneret plate having a filament-forming orifice formed therethrough for producing a filament in accordance with the present invention, the view being taken in a plane perpendicular to the central axis of the filament-forming orifice with the orifice having rounded end contour regions and concave sides;
Figure 2B is an end view, similar to the view of Figure 2A, showing an alternate embodiment of a spinneret plate for producing a filament in accordance with the present invention, the filament-forming orifice having rounded end contour regions and linear sides;
Figure 3A is an end view an alternate embodiment of a spinneret plate generally similar to that shown in Figure 2A in that the orifice has concave sides, but with end contour regions each comprising at least two linear edges;
Figure 3B is an end view an alternate embodiment of a spinneret plate generally similar to that shown in Figure 2B in that the orifice has linear sides, but with end contour regions each comprising at least two linear edges;
Figure 4 is stylized diagrammatic illustration of a spinning arrangement that utilizes a spinneret plate as shown in Figures 2A, 2B, 2C, 3A or 3B for spinning filaments in accordance with the invention;
Figure 5 is stylized diagrammatic illustration of a carpet fabricated using filaments of the invention;
Figure 6A is stylized diagrammatic side sectional illustration of a rotating ball mill test chamber used to test filaments of the invention;
Figure 6B is a diagrammatic end view illustrating the operation of the ball mill test when testing filaments of the present invention;
Figures 7A and 7B are photographs illustrating a comparative trilobal cross section filament before and after fibrillation testing using the rotating ball mill test chamber of Figure 6A;
Figures 8A and 8B are photographs illustrating a comparative round cross section filament before and after fibrillation testing using the rotating ball mill test chamber of Figure 6A; and
Figures 9A and 9B are photographs illustrating a filament in accordance with the present invention before and after fibrillation testing using the rotating ball mill test chamber of Figure 6A.

### DETAILED DESCRIPTION OF THE INVENTION

Throughout the following detailed description similar reference numerals refer to similar elements in all figures of the drawings.

Figure 1 is a cross-section view through a solid core, fibrillation-resistant, synthetic polymeric filament 10 in accordance with one aspect of the present invention, taken in a plane substantially perpendicular to the central longitudinal axis 10A of the filament.

The filament 10 is preferably fabricated from a polytrimethylene terephthalate polymeric material. More preferably, the poly-trimethylene terephthalate polymeric material wherein the 1,3 propane diol is biologically produced, although it should also be understood that the 1,3 propane diol derived via a petroleum route may also used in combination with biologically based 1,3 propane diol.

The polymeric material may be pigmented with a solution dyed color additive or a delusterant such as TiO2. Alternatively, the polymeric material may be non-pigmented for later dying. The polymeric material may contain UV stabilizer(s), anti-oxidant(s) and/or other performance-improving additive(s) (including flame retardant(s), such as phosphorus- and/or nitrogen-containing compound(s); toughening agent(s); and/or nucleation-inhibiting agent(s).

The filament may also be fabricated from other polymeric materials, such as polyester, nylon, polypropylene and blends thereof.

As seen from Figure 1 the filament 10 is, in the cross section plane perpendicular to its axis, three-sided in form. The sides 12¹, 12², 12³ are substantially equal in length. Each side 12¹, 12², 12³ is generally convex in shape with a mid-point 12M¹, 12M², 12M³ therealong. Each side 12¹, 12², 12³ lies on a respective circle of curvature having a radius 12R¹, 12R², 12R³. Each circle of curvature is centered on a respective center point 12C¹, 12C², 12C³. The center points 12C¹, 12C², 12C³ each lie on a respective reference radius emanating from the axis 10A of the filament 10.

Each respective side 12¹, 12², 12³ meets with a side adjacent thereto through a substantially rounded tip 14¹, 14², 14³, respectively. The rounded contour of each tip 14¹, 14², 14³ lies on a circle of curvature centered on a respective center point 16¹, 16², 16³. The radius of the circle of curvature of the tips 14¹, 14², 14³ is indicated by the reference character "b". Each center of curvature 16¹, 16², 16³ is itself spaced by a predetermined distance "a" from the central axis 10A of the filament. Only one center of curvature (16¹) is shown for clarity of illustration

The outermost point of each tip 14¹, 14², 14³ of the filament 10 lies on a circumscribed circle 24 having a radius substantially equal to a length (a + b). The midpoint 12M¹, 12M², 12M³ of each respective side 12¹, 12², 12³ lies on an inscribed circle 26 centered on the central axis 10A of the filament 10. The radius of the inscribed circle 26 is substantially equal to a length "c". Accordingly, the filament 10 exhibits a modification ratio ("MR") defined by the ratio of the radius (a+b) of the circumscribed circle to the radius (c) of the inscribed circle, thus: $M ⁢ R = \left(a+b\right) / c .$

Mathematical modeling of filaments having trilobal cross-section shows that lobes and the sides are susceptible to failure under compressive, bending and/or torsion loads. The effect of these stresses acting upon the filaments result in fibrillation and the corresponding texture degradation of the filament during wear.

Analyses also indicate that maximum bending stress is imposed on the end contour regions of the filament, while maximum torsion and compression forces are imposed substantially centrally along the sides of the filament. For example, the compressive stress ("σ") at the contact point between two adjacent filaments has been found to be inversely proportional to the square root of filament diameter "d" when filaments are parallel to each other,
thus, σ = d^{-½}.

In the case where the filaments are perpendicular to each other, the compressive stress ("σ") is inversely proportional to the 2/3^{rd} power of filament diameter, thus, σ = d^{½}.

As will be developed it is believed that the fiber geometry disclosed by this invention reduces these stress levels, resulting in a filament having improved fibrillation resistant properties. Filaments in accordance with the present invention are believed to overcome weaknesses of round as well as trilobal cross-sections under various loading conditions.

In particular, it has been found that forming a filament with more robust end contours and more robust filament tip region will counteract bending stress imposed on the filament. If the radius of the circle of curvature of the tips 14¹, 14², 14³ is kept large stress levels at tips are lowered below the levels occurring at the lobes of a trilobal cross-section.

Likewise, as opposed to filaments having a round cross-section, configuring the filament with flatter, less concave sides result in filaments more able to retain their shape in the face of forces imposed by use. Filaments with large radii 12R¹, 12R², 12R³ relative to the diameter of a round filament having an equivalent cross-sectional area lead to a substantial reduction in the compressive contact stress over round filaments.

Accordingly, filaments in accordance with the present invention exhibit various dimensional parameters and certain relationships therebetween, as follows:
the filament has a denier-per-filament ("dpf") in the range 10 < "dpf" < 35;
the distance "a" lies in the range 0.0003 inches (6 micrometers) < "a" < .004 inches (102 micrometers);
the distance "b" lies in the range from 0.00008 inches (2 micrometers) < "b" < .0001 inches (24 micrometers);
the distance "c" lies in the range from 0.0003 inches (8 micrometers) < "c" < .0025 inches (64 micrometers); and
the modification ratio ("MR") lies in the range from about 1.1 < "MR" < about 2.0.

In a more preferred instance:
the filament has a denier-per-filament ("dpf") in the range 12 < "dpf" < 32;
the distance "a" lies in the range 0.00035 inches (9 micrometers) < "a" < 0.003 inches (76 micrometers);
the distance "b" lies in the range from 0.00010 inches (3 micrometers) < "b" < .00095 inches (25 micrometers);
the distance "c" lies in the range from 0.0005 inches (10 micrometers)< "c" < .002 inches (51 micrometers); and
the modification ratio ("MR") lies in the range from about 1.1 < "MR" < about 2.0.

Preferably, the filament has a tenacity greater than 1.5 grams per denier.

In another aspect the present invention is directed to a spinneret plate 100 for forming a solid core, fibrillation-resistant, synthetic polymeric filament. The plate 100 is a relatively massive member having a plurality of filament-forming orifices 102 provided therethrough. Each orifice has a center 102A. The plate 100 may be fabricated from a material such as stainless steel. Suitable grades of stainless steel include 440C, 316, 17-4 PH, 430, or Carpenter 20. The steel grade selected should be free of internal defects. Typically the orifices are formed through the plate 100 using machining technology such as laser cutting or electrical discharge machining.

An enlarged view of a portion of the surface of a spinneret plate 100 and one of the orifices 102 formed therein is shown Figures 2A, 2B, 3A and 3B. Each of these Figures illustrates one of the various alternative configurations of an single orifice 102 in accordance with various embodiments of the present invention.

In general, for each embodiment of this aspect of the invention a filament-forming orifice 102 is an aperture having three substantially equal length sides 112¹, 112², 112³. The midpoint 112M¹, 112M², 112M³ of each side lies on an inscribed circle 113 having a radius "H" centered on the center point 102A of the orifice. Each of the sides 112¹, 112², 112³ terminates in a first and a second end point, respectively indicated in the drawings by the Roman numerals I, II.

The first end point I of any one side is connected to the second end point II of an adjacent side by an end contour 114, 114' . The end contour 114, 114' in each of the embodiments of Figures 2A, 2B and Figures 3A and 3B take alternative forms.

In the embodiments illustrated in Figures 2A and 2B the end contour 114 takes the form of a circle centered on center point 116 and having a radius of the dimension "C". Each center point 116 is spaced a predetermined distance "D" along a reference radius 120 emanating from the center 102A of the orifice. The outermost point on each circular end contour 114 lies on a circumscribed circle 121 centered on the center 102A of the orifice and having a radius "(C+D)". The first end point I of any one side and the second end point II of an adjacent side are spaced from each other by a chord 122 of the circular end contour. Each end point I, II defines a point of tangency of the circular end contour 114.

The modification ratio ("MR") of an orifice is defined as the ratio of the radius of a circumscribed circle of the orifice to the radius of the inscribed circle of the orifice.

In a preferred implementation of this embodiment of the invention shown in Figures 2A and 2B:
the distance "C" lies in the range 0.0015 inches (38 micrometers) < "C" < .0040 inches (102 micrometers);
the distance "D" lies in the range from 0.0150 inches (381 micrometers) < "D" < .0300 inches (762 micrometers) .

In a more preferred case:
the distance "C" lies in the range 0.0020 inches (51 micrometers) < "C" < .0035 inches (89 micrometers);
the distance "D" lies in the range from 0.0175 inches (445 micrometers) < "D" < .0280 inches (711 micrometers).

Alternatively, in the embodiments illustrated in Figures 3A and 3B, each end contours 114' is defined by at least two linear edges 126A, 126B. Any convenient number of linear edge segments may be used to define an end contour 114'. In these embodiments the first end point I of any one side and the second end point II of an adjacent side are spaced from each other by a baseline 128 having a length "2F". Each baseline 128 lies a predetermined distance "G" on the reference radius 120. The linear edges 126A, 126B of the contour 114' intersect each other at an apex 130 also lying on the reference radius 120. The apex 130 is spaced a distance "E" from the baseline 128.

The apex 130 of each end contour 114' lies on a circumscribed circle 121 centered on the center 102A of the orifice. In these Figures the circumscribed circle 121 has a radius " (G+E) ".

In accordance with this embodiment of the invention shown in Figures 3A and 3B:
the distance "E" lies in the range 0.0025 inches (64 micrometers) < "E" < .0150 inches (381 micrometers);
the distance "F" lies in the range from 0.0015 inches (38 micrometers) < "F" < .0040 inches (102 micrometers); and
the distance "G" lies in the range from 0.0150 inches (381 micrometers) < "G" < .0300 inches (762 micrometers).
More preferably:
the distance "E" lies in the range 0.0030 inches (76 micrometers) < "E" < .0100 inches (254 micrometers);
the distance "F" lies in the range from 0.0020 inches (51 micrometers) < "F" < .0035 inches (89 micrometers); and
the distance "G" lies in the range from 0.0175 inches (445 micrometers) < "G" < .0280 inches (711 micrometers).

The orifices 102 as illustrated in Figures 2A and 3A also differ from those shown in Figures 2B and 3B in the form taken by the sides 112.

In the embodiments of Figures 2A and 3A the sides 112¹, 112², 112³ are generally concave in shape and lie along a circle of curvature centered on a respective center of curvature 112C¹, 112C², 112C³. Each center of curvature 112C¹, 112C², 112C³ is located on a reference line 134 emanating radially from the central axis 102A of the orifice. The radius of the circle of curvature has a dimension indicated by the reference character "B". Each center of curvature 112C¹, 112C², 112C³ is located a predetermined distance "A" from the central axis 102A. It should be noted that the radius "H" of the inscribed circle 113 is equal to (A - B).

For orifices having concave sides as shown in Figures 2A and 3A the following additional dimensional constraints apply:
the distance "A" lies in the range 0.0300 inches (762 micrometers) < "A" < .0900 inches (2286 micrometers);
the distance "B" lies in the range from 0.0200 inches (508 micrometers) < "B" < .0800 inches (2032 micrometers);
the ratio (A/B) lies within the range from about 1.0 < (A/B) < about 1.6; and
the modification ratio ("MR") lies in the range from about 1.5 < "MR" < about 4.5.

More preferably:
the distance "A" lies in the range 0.0300 inches (762 micrometers) < "A" < .0800 inches (2032 micrometers);
the distance "B" lies in the range from 0.0200 inches (508 micrometers) < "B" < .0700 inches (1778 micrometers);
the ratio (A/B) lies within the range from about 1.1 < (A/B) < about 1.5; and
the modification ratio ("MR") lies in the range from about 1.8 < "MR" < about 3.5.

For orifices having concave sides (Figures 2A and 3A) the modification ratio ("MR") lies in the range from about 2.0 < "MR" < about 4.0. More preferably, the modification ratio ("MR") lies in the range from about 2.2 < "MR" < about 3.5.

As the radius of the circle of curvature of the side of the orifice is increased the contour of the side flattens, until at a very large radius the side becomes close to linear.

For orifices having linear sides and circular end contours (Figures 2B) the distance "H" (i.e., the radius of the inscribed circle) lies in the range from 0.0090 inches (229 micrometers) < "H" < 0.0190 inches (483 micrometers). The modification ratio ("MR") lies in the range from about 1.6 < "MR" < about 2.5. More preferably, the distance "H" lies in the range from 0.0108 inches (274 micrometers) < "H" < 0.0175 inches (445 micrometers) and the modification ratio ("MR") lies in the range from about 1.7 < "MR" < about 2.3.

For orifices having linear sides and linear end contours (Figures 3B) the distance "H" (i.e., the radius of the inscribed circle) lies in the range from 0.0088 inches (224 micrometers) < "H" < 0.0185 inches (470 micrometers). The modification ratio ("MR") lies in the range from about 1.6 < "MR" < about 2.5. More preferably, the distance "H" lies in the range from 0.0105 inches (267 micrometers) < "H" < 0.0170 inches (432 micrometers) and the modification ratio ("MR") lies in the range from about 1.7 < "MR" < about 2.3.

Figure 4 is stylized diagrammatic illustration of a spinning arrangement generally indicated by the reference character 200 for manufacturing bulked continuous filaments of present invention. Polymer melt is pumped through spin pack assembly 202 that includes a spinneret plate 100 having a plurality of orifices 102 shaped in accordance with this invention. The spin pack assembly 202 may also contain a filtration medium.

Filaments 10 of desired shapes are obtained when polymer is extruded through the spinneret plate 100 and filaments are pulled through a quench chimney 204 by feed rolls 206. Finish is applied to the filaments 10 for downstream processability by a finish roll 208 located prior to the feed rolls 206. The feed rolls 206 are kept at the room temperature or maintained at a temperature above polymer glass transition temperature to effectively draw and orient molecules during the draw process. Draw rolls 210, running at a predetermined speed faster than the feed rolls 206 by the amount of the draw ratio, are heated to a temperature above the glass transition temperature and below the melting point of the polymer to anneal the drawn fiber. At this point the filaments may be collected by a winder 212 through a let down roll 214 or continue for further processing. In an alternate arrangement, a set of heated pre-draw rolls may be employed between the finish applicator 208 and feed rolls 206. This arrangement provides additional flexibility of imparting suitable temperature and tension history to filaments to optimize draw between roll sets 206 and 210.

A bulking jet 220 employing hot air or steam is used to impart a random, three-dimensional curvilinear crimp to the filaments. The resulting bulked filaments are laid on to a rotating drum 224 having a perforated surface. The filaments are cooled under zero tension by pulling air through them using a vacuum pump. Water may additionally be misted onto the filaments on the drum 224 to facilitate cooling. After the filaments have been cooled below the glass transition temperature, filaments are pulled off the drum 224. If desired another finish for mill processing may applied by finish roll 226. The filament bundle is interlaced periodically by an interlacing jet 230 disposed between a pull roll 232 and a let down roll 234, and collected by a winder 236.

Figure 5 is stylized diagrammatic illustration of a carpet generally indicated by the reference character 300 having tufted with yarn 302 made from filaments 10 of the present invention. In the embodiment illustrated the yarn 302 is formed from two twisted and heat-set filaments. Alternatively, the yarn could be formed by air-entangling filaments 10 or the yarn could be directly tufted without twisting or entanglement.

The yarn is tufted through a primary backing 304 to form pile tufts 306. The pile tufts 306 may take the level loop form shown in Figure 5. Alternatively, the pile tufts may be multi-level loop, berber, plush, saxony, frieze or sheared form.

The carpet 300 is completed by a secondary 308 adhered to the primary backing 304 using an adhesive 310.

Other potential end uses of the filaments of the present invention include luggage, handbags, automotive fabrics.

Figure 6A is a stylized diagrammatic illustration, taken in side section, of a rotating ball mill test chamber 400 used to test filaments 10 of the invention. Figure 6B is a diagrammatic end view illustrating the operation of the ball mill test when testing filaments of the present invention.

The test chamber 400 comprises a cylindrical barrel 402 closed at one end by an integral base 404. The opposite end of the barrel 402 receives a lid 406. The lid 406 is secured to the rim of the barrel 402 by bolts 408. Both the base 404 and the lid 406 have an array of axially aligned mounting apertures 410 formed therein.

Access to the interior of the barrel 402 is afforded through a port opening 412 provided in the center of the lid 406. The port opening 412 is closed by a removable hatch 416. The hatch 416 is secured to the lid 406 by a screws 418.

To prepare the chamber for a test, bundles of filaments 10 under test are strung between the base 404 and the lid 406 using the mounting apertures 410. The filaments under test may be conveniently secured to the surfaces of the base 404 and the lid 406, as by tape. Any convenient number of ball bearings 420 (Figure 6B) are introduced into the chamber through the port opening 412 and the hatch 416 secured. Nine millimeter (9 mm) stainless steel ball bearings may be used.

The dynamics of a filament test using the test chamber 400 are illustrated in Figure 6B. The test chamber 400 is placed on two driven bars 424A, 424B of a rotating mill apparatus, such as a device manufactured by U.S. Stoneware, a division of E.R. Advanced Ceramics, East Palatine, Ohio. As the bars 424 are rotated in the direction 428 the bearings 420 impinge on the filaments 10 strung axially across the interior of the barrel. The test may be conducted for any convenient time period at a nominal rotational speed of one hundred rpm, although other speeds in the range from about 30 to about 120 rpms may be suitable employed.

Fiber cross-section images of the filaments tested using the test chamber 400 indicate fibrillation damage to the filaments that is similar to the fibrillation damage done to filaments of a carpet subjected to any of the various industry standard test methods used to measure texture retention. The similarity of fibrillation damage lends confidence to conclusions regarding the fibrillation resistance of filaments tested using the chamber 400.

### EXAMPLES

Example 1 (Comparative) Using a spinning arrangement as shown in Figure 4 bio-based poly-trimethylene terephthalate polymer having an intrinsic viscosity of 1.02 and less than 50 ppm moisture was spun through a 17-hole spinneret suitable for trilobal cross-section filaments. The temperature set points for downstream barrels of the 28-mm Warner & Pfleiderer twin extruder, transfer line, pumps, pack and die were in the range of 268-270°C. The spinning throughput was 60 grams per minute. The molten filaments were cooled in the chimney, where the room air was blown past the filaments using a profiled quench with air velocity in the range of 21-30 feet per minute as a function of distance from the spinneret face with higher velocity near the spinneret. Filaments were pulled by a pair of feed rolls at 60°C at a surface speed of 600 meters per minute through the quench zone. Filaments were coated with a lubricant immediately prior to the feed roll. The coated filaments were drawn by a draw ratio of 3 and annealed by a pair of rolls heated to 160°C with a surface speed of 1800 meters/minute. The filaments were then wound.

Filaments produced had the following properties:
Denier per filament = approximately 18
MR = 2.1
Arm angle = 22°
Tenacity of yarn, as produced, was 2.02 gm/denier.

Two hundred sixty filaments were strung through the rotating ball mill test chamber 400, described earlier, under a tension of approximately 20 gm without imparting any substantial twist to the yarn bundle. One hundred 9 mm stainless steel ball bearings were placed in the chamber. The test was conducted for 16 hours at 100 rpm.

Cross-sectional images of yarn bundles were obtained before and after the 16 hour test using a Hardy plate and an optical microscope and are shown in Figure 7A and 7B, respectively.

Example 2 (Comparative) Using a spinning arrangement as shown in Figure 4 bio-based poly-trimethylene terephthalate polymer having an intrinsic viscosity of 1.02 and less than 50 ppm moisture was spun through a 34-hole spinneret suitable for round cross-section filaments. The temperature set points for downstream barrels of the 28-mm Warner & Pfleiderer twin extruder, transfer line, pumps, pack and die were in the range of 268-270°C. The spinning throughput was 88.1 grams per minute. The molten filaments were cooled in the chimney, where the room air was blown past the filaments using a profiled quench with air velocity in the range of 21-30 feet per minute as a function of distance from the spinneret face with higher velocity near the spinneret. Filaments were pulled by a pair of feed rolls at 60°C at a surface speed of 415 meters per minute through the quench zone. Filaments were coated with a lubricant immediately prior to the feed roll. The coated filaments were drawn by a draw ratio of 3.25 and annealed by a pair of rolls heated to 160°C with a surface speed of 1350 meters/minute. The filaments were then wound. Denier per filament was approximately 18. Tenacity of yarn, as produced, was 2.75 gm/denier.

Two hundred seventy two filaments were strung through the rotating ball mill test chamber 400, described earlier, under a tension of approximately 20 gm without imparting any substantial twist to the yarn bundle. One hundred 9 mm stainless steel ball bearings were placed in the device. The test was conducted for 16 hours at 100 rpm. Cross-section images of yarn bundles were obtained before and after the 16 hour test using a Hardy plate and an optical microscope and are shown in Figure 8A and 8B, respectively.

Example 3 Using a spinning arrangement as shown in Figure 4 bio-based poly-trimethylene terephthalate polymer having an intrinsic viscosity of 1.02 and less than 50 ppm moisture was spun through a 10-hole spinneret of present invention with following dimensions (Figure 3A):
A = 0.066 inch, (1680 micrometers)
B = 0.0554 inch, (1410 micrometers)
F = 0.0028 inch, (71.1 micrometers)
G = 0.0225 inch, (572 micrometers)
E = 0.0047 inch, (119 micrometers)
A/B = 1.19,
2F/G = 0.249,
E/D = 0.21,
modification ratio MR = 2.6.

The temperature set points for downstream barrels of the 28-mm Warner & Pfleiderer twin extruder, transfer line, pumps, pack and die were in the range of 268-270°C. The spinning throughput was 30 grams per minute. The molten filaments were cooled in the chimney, where the room air was blown past the filaments using a profiled quench with air velocity in the range of 21-30 feet per minute as a function of distance from the spinneret face with higher velocity near the spinneret. Filaments were pulled by a pair of feed rolls at 60°C at a surface speed of 500 meters per minute through the quench zone. Filaments were coated with a lubricant immediately prior to the feed roll. The coated filaments were drawn by a draw ratio of 3 and annealed by a pair of rolls heated to 160°C with a surface speed of 1500 meters/minute. The filaments were then wound.

Filaments produced had the following properties:
Denier per filament = approximately 18
a = 0.00083 inch (21.1 micrometers)
b = 0.00025 inch (6.35 micrometers)
c = 0.00077 inch (19.6 micrometers)
MR = 1.406
Tenacity of yarn, as produced, was 1.99 gm/denier.

Two hundred sixty filaments were strung through the rotating ball mill test chamber 400, described earlier, under a tension of approximately 20 gm without imparting any substantial twist to the yarn bundle. One hundred 9 mm stainless steel ball bearings were placed in the device. The test was conducted for 16 hours at 100 rpm. Cross-section images of yarn bundles were obtained before and after the 16 hour test using a Hardy plate and an optical microscope and are shown in Figure 9A and 9B, respectively.

Fibrillation-resistant behavior of cross-section of a filament in accordance with the present invention is easily seen from comparison of the image in Figure 9B with the images of the comparative examples shown in Figures 7B and 8B. Comparing Figures 7A and 7B, bending and severing of the lobes, indicating excessive fibrillation is easily seen. Similarly, there is excessive deformation of filaments having round cross-section as seen from Figures 8A and 8B. By contrast, very little deformation is seen in Figure 9B when compared to as-produced filaments before the ball mill test, shown in Figure 9A.

Example 4 (Comparative) Using a spinning arrangement as shown in Figure 4 bio-based poly-trimethylene terephthalate polymer having an intrinsic viscosity of 1.02 and less than 50 ppm moisture was spun through a 68-hole spinneret for trilobal cross-section.

The temperature set points for downstream barrels of a single screw extruder, transfer line, pumps, pack and die were in the range of 230-260°C. The spinning throughput was 466.7 grams per minute. The molten filaments were cooled in the chimney, where the 16°C air was blown past the filaments. Filaments were pulled by a pair of feed rolls at 38°C at a surface speed of 1900 meters per minute through the quench zone. Filaments were coated with a lubricant immediately prior to the feed roll. The coated filaments were pre-drawn by a ratio of 1.01 by a pair of rolls at 50°C with a surface speed of 1920 meters per minute. The filaments were then drawn by a ratio of 1.98 and annealed by another pair of heated draw rolls at 165°C running at a surface speed of 3800 meters per minute. The filaments were texturized using a stuffer-jet bulker with jet air temperature at 225 °C, interlaced and wound at 3170 meters per minute.

Filaments produced had the following properties:
Denier per filament = approximately 19.5
Trilobal cross-section with MR = 1.85
Tenacity of yarn, as produced, was 2.2 gm/denier.

Two ends were twisted at 4.75 twists/inch and heatset to stabilize twisted structure prior to tufting and finishing to produce 10^{th} gauge, 0.22 inch pile height carpet having a basis weight of approximately 24 oz/sq. yd. The carpet tested for wear had the following ratings:

### Hexapod (ASTM D5252)

4.0 after 4000 cycles and 2.3 after 12000 cycles Vetterman Drum (ASTM D5417)

4.7 after 5000 cycles and 2.8 after 22000 cycles.

Example 5 Using a spinning arrangement as shown in Figure 2B bio-based poly-trimethylene terephthalate polymer having an intrinsic viscosity of 1.02 and less than 50 ppm moisture was spun through a 70-hole spinneret of present invention with following dimensions (Figure 2B):
C = 0.0028 inch, (71.1 micrometers)
D = 0.0222 inch, (564 micrometers)
H = 0.0139 inch, (353 micrometers)
Modification ratio MR = 1.8

The temperature set points for downstream barrels of a single screw extruder, transfer line, pumps, pack and die were in the range of 245-260°C. The spinning throughput was 385 grams per minute. The molten filaments were cooled in the chimney, where the 17°C air was blown past the filaments. Filaments were pulled by a pair of feed rolls at 50°C at a surface speed of 1180 meters per minute through the quench zone. Filaments were coated with a lubricant immediately prior to the feed roll. The coated filaments were pre-drawn by a ratio of 1.008 by a pair of rolls at 55°C with a surface speed of 1190 meters per minute. The filaments were then drawn by a ratio of 2.52 and annealed by another pair of heated draw rolls at 160°C running at a surface speed of 3000 meters per minute. The filaments were texturized using a stuffer-jet bulker with jet air temperature at 205 °C, interlaced and wound at 2435 meters per minute.

Filaments produced had the following properties:
Denier per filament = approximately 20
a = 0.00085 inch (21.6 micrometers)
b = 0.00029 inch (7.37 micrometers)
c = 0.00091 inch (23.1 micrometers)
MR = 1.41

Tenacity of yarn, as produced, was 2.20 gm/denier.Two ends were twisted at 4.75 twists/inch and heatset to stabilize twisted structure prior to tufting and finishing to produce 10^{th} gauge, 0.22 inch pile height carpet having a basis weight of approximately 24 oz/sq. yd. The carpet tested for wear had the following ratings:

### Hexapod (ASTM D5252)

4.5 after 4000 cycles and 3.7 after 12000 cycles Vetterman Drum (ASTM D5417)
4.5 after 5000 cycles and 3.5 after 22000 cycles.

Example 6 Using a spinning arrangement as shown in Figure 2B bio-based poly-trimethylene terephthalate polymer having an intrinsic viscosity of 1.02 and less than 50 ppm moisture was spun through a 70-hole spinneret of present invention with following dimensions (Figure 2A):
A = 0.0759 inch, (1930 micrometers)
B = 0.0637 inch, (1620 micrometers)
C = 0.0032 inch, (81.3 micrometers)
D = 0.0222 inch, (564 micrometers)
Modification ratio MR = 2.4

The temperature set points for downstream barrels of a single screw extruder, transfer line, pumps, pack and die were in the range of 245-260°C. The spinning throughput was 385 grams per minute. The molten filaments were cooled in the chimney, where the 17°C air was blown past the filaments. Filaments were pulled by a pair of feed rolls at 50°C at a surface speed of 1180 meters per minute through the quench zone. Filaments were coated with a lubricant immediately prior to the feed roll. The coated filaments were pre-drawn by a ratio of 1.008 by a pair of rolls at 55°C with a surface speed of 1190 meters per minute. The filaments were then drawn by a ratio of 2.52 and annealed by another pair of heated draw rolls at 160°C running at a surface speed of 3000 meters per minute. The filaments were texturized using a stuffer-jet bulker with jet air temperature at 205 °C, interlaced and wound at 2435 meters per minute.

Filaments produced had the following properties:
Denier per filament = approximately 20
a = 0.00087 inch (22.1 micrometers)
b = 0.00033 inch (8.38 micrometers)
c = 0.00084 inch (21.3 micrometers):
MR = 1.43
Tenacity of yarn, as produced, was 1.95 gm/denier.

Two ends were twisted at 4.75 twists/inch and heatset to stabilize twisted structure prior to tufting and finishing to produce 10^{th} gauge, 0.22 inch pile height carpet having a basis weight of approximately 24 oz/sq. yd. The carpet tested for wear had the following ratings:

### Hexapod (ASTM D5252)

4.5 after 4000 cycles and 3.7 after 12000 cycles Vetterman Drum (ASTM D5417)
4.5 after 5000 cycles and 3.8 after 22000 cycles.

Fibrillation-resistant behavior of the cross section of a filament in accordance with the present invention is further exemplified by comparison of the wear performance of carpets in Examples 5 and 6 of the present invention with a typically used trilobal cross-section described in Example 4. Both Hexapod and Vetterman drum tests showed superior long-term performance (12000 cycles and 22000 cycles, respectively) of carpets made in accordance with the present invention. As shown in Table 1 below, the "Difference" between the values for both the Hexapod and Vetterman Drum tests for Examples 5 and 6 of the present invention at the 12000 and 22000 cycle test points were higher than the "Differences" for Example 4 (Comparative) at the same 12000 and 22000 cycle test points. These data indicate better fibrillation resistance for Examples 5 and 6 than for Example 4.

**Table 1**

| Ex. No. | Hexapod 4000 cycles (Q) | Hexapod 12000 Cycles (R) | Difference for Hexapod (Q - R) | Vetterman Drum 5000 Cycles (X) | Vetterman Drum 22000 Cycles (Y) | Difference For Vetterman Drum (X - Y) |
|---|---|---|---|---|---|---|
| 4 (comp | 4.0 | 2.3 | 1.7 | 4.7 | 2.8 | 1.9 |
| 5 | 4.5 | 3.7 | 0.8 | 4.5 | 3.5 | 1.0 |
| 6 | 4.5 | 3.7 | 0.8 | 4.5 | 3.8 | 0.7 |

## Claims

1. A solid core, fibrillation-resistant, synthetic polymeric filament having a
longitudinal axis extending therethrough and a three-sided cross section in a plane perpendicular to the longitudinal axis,
the sides being substantially equal in length and convex in form, each side having a midpoint therealong, each midpoint lying on an inscribed circle centered on the central axis of the filament, the inscribed circle having a radius substantially equal to a length "c",
each side meeting an adjacent side through a substantially rounded tip centered on a respective circle of curvature, each circle of curvature having a radius substantially equal to a length "b", each circle of curvature being spaced from the axis of the filament by a distance "a", each tip of the filament lying on a circumscribed circle having a radius substantially equal to a length (a+b),
the filament having a modification ratio (MR) defined by the ratio of the radius (a+b) of the circumscribed circle to the radius (c) of the inscribed circle, wherein
the filament has a denier-per-filament ("dpf') in the range 10<"dpf"<35;
the distance "a" lies in the range 0.00025 inches (6 micrometers)<"a"<0.004 inches (102 micrometers);
the distance "b" lies in the range from 0.00008 inches (2 micrometers) <"b"<0.0010 inches (24 micrometers);
the distance "c" lies in the range from 0.0003 inches (8 micrometers) <"c"<0.0025 inches (64 micrometers); and
the modification ratio ("MR") lies in the range from about 1.1 <"MR" < about 2.0, wherein the synthetic polymer is poly-trimethylene terephthalate.

2. A carpet having a backing and a plurality of tufts attached to the backing,
each tuft having a solid core, fibrillation-resistant, synthetic polymeric filament as claimed in claim 1.

3. The filament or carpet of claims 1 or 2 wherein the filament has a tenacity greater than 1.5 grams per denier.

4. The filament or carpet of claims 1 or 2 wherein
the filament has a denier-per-filament ("dpf") in the range 12<"dpf"<32;
the distance "a" lies in the range 0.00035 inches (9 micrometers)<"a"<0.003 inches (76 micrometers);
the distance "b" lies in the range from 0.00010 inches (3 micrometers) <"b"<0.00095 inches (25 micrometers);
the distance "c" lies in the range from 0.0005 inches (10 micrometers) <"c"<0.002 inches (51 micrometers); and
the modification ratio ("MR") lies in the range from about 1.1 <"MR" < about 2.0.

5. The filament or carpet of claim 1 wherein the poly-trimethylene terephthalate has a delusterant therein.

6. The filament or carpet of claim 1 wherein the poly-trimethylene terephthalate is pigmented.

7. The filament or carpet of claim 1 wherein the poly-trimethylene terephthalate has a 1,3 propane diol that is biologically produced.

8. The filament or carpet of claim 1 wherein the poly-trimethylene terephtalate has a flame retardant therein.

9. A spinneret plate for forming a solid core, fibrillation-resistant, synthetic polymeric filament having a longitudinal axis extending therethrough and a three-sided cross section in a plane perpendicular to the longitudinal axis,
the spinneret plate having a plurality of orifices formed therein, each orifice having a center and three sides, each side terminating in a first and a second end point, each side having a midpoint between the first and second end points,
the first end point of one side being connected to the second end point of an adjacent side by a circular end contour, the circular end contour having a radius equal to a dimension "C" measured from a center point lying on a radial line emanating from the center of the orifice, the center point of each end contour being disposed a predetermined distance "D" from the center of the orifice,
the first end point of each side being spaced from the second end point of an adjacent side along a chord defined between the end points of adjacent sides, and,
a point on each circular end contour lying on a circumscribed circle having a radius "(C+D)" centered on the center of the orifice, the midpoints of each side lying on an inscribed circle having a radius "H" centered on the center of the orifice, wherein
the distance "C" lies in the range 0.0015 inches (38 micrometers) <"C"<0.0040 inches (102 micrometers);
the distance "D" lies in the range from 0.0150 inches (381 micrometers) <"D"<0.0300 inches (762 micrometers).

10. The spinneret plate of claim 9 wherein
the distance "C" lies in the range 0.0020 inches (51 micrometers) <"C"<0.0035 inches (89 micrometers);
the distance "D" lies in the range from 0.0175 inches (445 micrometers) <"D"<0.0280 inches (711 micrometers).

11. The spinneret plate of claim 9 wherein each end point of each side is a point of tangency of a circular end contour.

12. The spinneret plate of claim 9 wherein
each side of each orifice is substantially concave with each side lying on a reference circle having a center located on a reference radius emanating from the center point of the orifice and passing through a midpoint of a side,
the center of the reference circle being disposed a predetermined distance "A" along the reference radius from the central axis of the orifice, the reference circle having a radius of dimension "B",
the orifice has a modification ratio ("MR") defined by the ratio of the radius (C+D) of the circumscribed circle to the radius "(A-B)" of the inscribed circle, thus, $ʺMRʺ = \left(C+D\right) / ʺHʺ ,$
wherein
the distance "A" lies in the range 0.0300 inches (762 micrometers) <"A"<0.0900 inches (2286 micrometers);
the distance "B" lies in the range from 0.0200 inches (508 micrometers) <"B"<0.0800 inches (2032 micrometers);
the ratio (A/B) lies within the range from about 1.0<(A/B)< about 1.6; and
the modification ratio ("MR") lies in the range from about 1.5<"MR" < about 4.5.

13. The spinneret plate of claim 12 wherein
the distance "A" lies in the range 0.0300 inches (762 micrometers) <"A"<0.0800 inches (2032 micrometers);
the distance "B" lies in the range from 0.0200 inches (508 micrometers) <"B"<0.0700 inches (1778 micrometers);
the ratio (A/B) lies within the range from about 1.1<(A/B)< about 1.5; and
the modification ratio ("MR") lies in the range from about 1.8<"MR" < about 3.5.

14. The spinneret plate of claim 9 wherein each side of each orifice is substantially linear,
a point on each circular end contour lying on a circumscribed circle having a radius "(C+D)" centered on the center of the orifice,
the midpoints of each side lying on a inscribed circle having a radius "H" centered on the center of the orifice, wherein
the distance "H" lies in the range from 0.0090 inches (229 micrometers) <"H"<0.0190 inches (483 micrometers),
the orifice has a modification ratio ("MR") defined by the ratio of the radius (C+D) of the circumscribed circle to the radius "H" of the inscribed circle, thus, $ʺMRʺ = \left(C+D\right) / ʺHʺ ,$
wherein
the modification ratio ("MR") lies in the range from about 1.6<"MR" < about 2.5.

15. The spinneret plate of claim 14 wherein
the distance "H" (i.e., the radius of the inscribed circle) lies in the range from 0.0108 inches (274 micrometers)<"H"<0.0175 inches (445 micrometers)
the modification ratio ("MR") lies in the range from about 1.7<"MR" < about 2.3.

16. A spinneret plate for forming a solid core, fibrillation-resistant, synthetic polymeric filament having a longitudinal axis extending therethrough and a three-sided cross section in a plane perpendicular to the longitudinal axis,
the spinneret plate having a plurality of orifices formed therein, each orifice having a center and three sides, each side terminating in a first and a second end point, each side having a midpoint between the first and second end points,
the first end point of each side being spaced from the second end point of an adjacent side by a baseline defined between the end points of adjacent sides, the baseline intersecting with a reference radius emanating from the center point, the intersection point between the baseline and the reference radius lying a distance "G" along the reference radius from the center of the orifice, the baseline having a predetermined length "2F",
the first end point of one side being connected to the second end point of an adjacent side by an end contour having at least two linear edges, the linear edges intersecting in an apex, the apex being spaced from the intersection of the baseline and the reference radius by a dimension "E", wherein
the distance "E" lies in the range 0.0025 inches (64 micrometers) <"E"< .0150 inches (381 micrometers);
the distance "F" lies in the range from 0.0015 inches (38 micrometers) <"F"<0.0040 inches (102 micrometers); and
the distance "G" lies in the range from 0.0150 inches (381 micrometers) <"G"<0.0300 inches (762 micrometers).

17. The spinneret plate of claim 16 wherein
the distance "E" lies in the range 0.0030 inches (76 micrometers) <"E"<0.0100 inches (254 micrometers);
the distance "F" lies in the range from 0.0020 inches (51 micrometers) <"F"<0.0035 inches (89 micrometers); and
the distance "G" lies in the range from 0.0175 inches (445 micrometers) <"G"<0.0280 inches (711 micrometers).

18. The spinneret plate of claim 16 wherein
each side of each orifice is substantially concave with each side lying on a reference circle having a center located on a reference radius emanating from the center point of the orifice and passing through a midpoint of a side,
the center of the reference circle being disposed a predetermined distance "A" along the reference radius from the central axis of the orifice, the reference circle having a radius of dimension "B",
the orifice has a modification ratio ("MR") defined by the ratio of the radius (E+G) of the circumscribed circle to the radius "(E+G)" of the inscribed circle, thus, $ʺMRʺ = \left(C+D\right) / ʺ ⁢ \left(A-B\right) ⁢ ʺ ,$
wherein
the distance "A" lies in the range 0.0300 inches (762 micrometers) <"A"<0.0900 inches (2286 micrometers);
the distance "B" lies in the range from 0.0200 inches (508 micrometers) <"B"<0.0800 inches (2032 micrometers);
the ratio (A/B) lies within the range from about 1.0<(A/B)< about 1.6; and
the modification ratio ("MR") lies in the range from about 1.5<"MR" < about 4.5.

19. The spinneret plate of claim 18 wherein
the distance "A" lies in the range 0.0300 inches (762 micrometers) <"A"<0.0800 inches (2032 micrometers);
the distance "B" lies in the range from 0.0200 inches (508 micrometers) <"B"<0.0800 inches (1778 micrometers);
the ratio (A/B) lies within the range from about 1.1<(A/B)< about 1.5; and
the modification ratio ("MR") lies in the range from about 1.8<"MR" < about 3.5.

20. The spinneret plate of claim 16 wherein each side of each orifice is substantially linear,
the apex on each circular end contour lying on a circumscribed circle having a radius "(G+E)" centered on the center of the orifice,
the midpoints of each side lying on an inscribed circle having a radius "H" centered on the center of the orifice, wherein
the midpoints of each side lying on an inscribed circle having a radius "H" centered on the center of the orifice, wherein
the distance "H" lies in the range from 0.0088 inches (224 micrometers) <"H"<0.0185 inches (470 micrometers),
the orifice has a modification ratio ("MR") defined by the ratio of the radius (G+E) of the circumscribed circle to the radius "H" of the inscribed circle, thus, $ʺMRʺ = \left(G+E\right) / ʺHʺ ,$
wherein
the modification ratio ("MR") lies in the range from about 1.6<"MR"
< about 2.5.

21. The spinneret plate of claim 20 wherein
the distance "H" (i.e., the radius of the inscribed circle) lies in the range from 0.0105 inches (267 micrometers)<"H"<0.0170 inches (432 micrometers) the modification ratio ("MR") lies in the range from about 1.7<"MR"
< about 2.3.

22. A process for making a solid core, fibrillation-resistant, synthetic polymeric filament having a longitudinal axis extending therethrough and a three-sided cross section in a plane perpendicular to the longitudinal axis,
the sides being substantially equal in length and convex in form, each side having a midpoint therealong, each midpoint lying on an inscribed circle centered on the central axis of the filament, the inscribed circle having a radius substantially equal to a length "c",
each side meeting an adjacent side through a substantially rounded tip centered on a respective circle of curvature, each circle of curvature having a radius substantially equal to a length "b", each circle of curvature being spaced from the axis of the filament by a distance "a", each tip of the filament lying on a circumscribed circle having a radius substantially equal to a length (a+b),
the filament having a modification ratio (MR) defined by the ratio of the radius (a+b) of the circumscribed circle to the radius (c) of the inscribed circle, wherein
the filament has a denier-per-filament ("dpf") in the range 10<"dpf"<35;
the distance "a" lies in the range 0.00025 inches (6 micrometers)<"a"<0.004 inches (102 micrometers);
the distance "b" lies in the range from 0.00008 inches (2 micrometers) <"b"<0.0010 inches (24 micrometers);
the distance "c" lies in the range from 0.0003 inches (8 micrometers) <"c"<0.0025 inches (64 micrometers); and
the modification ratio ("MR") lies in the range from about 1.1 <"MR" < about 2.0.,
the process comprising the steps of:
a) pumping molten synthetic polymer through said spinneret plate of claim 11 and/or claim 18 having a plurality of orifices to form filaments wherein the synthetic polymer is poly-trimethylene terephthalate;
b) cooling the filaments;
c) applying a finish to the filaments;
d) drawing and annealing the filaments; and
e) bulking the filaments to impart a random, three-dimensional curvilinear crimp to the filaments.

23. The process of claim 22 wherein
each orifice of the spinneret plate has a center and three sides, each side terminating in a first and a second end point, each side having a midpoint between the first and second end points,
the first end point of one side being connected to the second end point of an adjacent side by a circular end contour, the circular end contour having a radius equal to a dimension "C" measured from a center point lying on a radial line emanating from the center of the orifice, the center point of each end contour being disposed a predetermined distance "D" from the center of the orifice,
the first end point of each side being spaced from the second end point of an adjacent side along a chord defined between the end points of adjacent sides, and,
a point on each circular end contour lying on a circumscribed circle having a radius "(C+D)" centered on the center of the orifice, the midpoints of each side lying on a inscribed circle having a radius "H" centered on the center of the orifice, wherein
the distance "C" lies in the range 0.0015 inches (38 micrometers) <"C"<0.0040 inches (102 micrometers);
the distance "D" lies in the range from 0.0150 inches (381 micrometers) <"D"<0.0300 inches 762 micrometers).

24. The process of claim 22 wherein
each orifice of the spinneret plate has a center and three sides, each side terminating in a first and a second end point, each side having a midpoint between the first and second end points,
the first end point of each side being spaced from the second end point of an adjacent side by a baseline defined between the end points of adjacent sides, the baseline intersecting with a reference radius emanating from the center point, the intersection point between the baseline and the reference radius lying a distance "G" along the reference radius from the center of the orifice, the baseline having a predetermined length "2F",
the first end point of one side being connected to the second end point of an adjacent side by an end contour having at least two linear edges, the linear edges intersecting in an apex, the apex being spaced from the intersection of the baseline and the reference radius by a dimension "E", wherein
the distance "E" lies in the range 0.0025 inches (64 micrometers) <"E"<0.0150 inches (381 micrometers);
the distance "F" lies in the range from 0.0015 inches (38 micrometers) <"F"<0.0040 inches (102 micrometers); and
the distance "G" lies in the range from 0.0150 inches (381 micrometers) <"G"<0.0300 inches (762 micrometers).

25. The process of claim 22 wherein the poly-trimethylene terephthalate has a 1,3 propane diol that is biologically produced.

## Patentansprüche

1. Fibrillierungsresistentes, synthetisches, polymeres Filament mit festem Kern, das eine Längsachse, die sich darin hindurch erstreckt, und einen dreiseitigen Querschnitt in einer zur Längsachse senkrechten Ebene aufweist,
wobei die Seiten im Wesentlichen längenmäßig gleich sind und eine konvexe Form aufweisen, wobei jede Seite einen Mittelpunkt daran entlang aufweist, wobei jeder Mittelpunkt auf einem Inkreis liegt, der auf die Mittelachse des Filaments zentriert ist, wobei der Inkreis einen Radius aufweist, der einer Länge "c" im Wesentlichen gleich ist,
wobei jede Seite auf eine benachbarte Seite durch eine im Wesentlichen abgerundete Spitze auftrifft, die auf einen entsprechenden Krümmungskreis zentriert ist, wobei jeder Krümmungskreis einen Radius aufweist, der einer Länge "b" im Wesentlichen gleich ist, wobei jeder Krümmungskreis von der Filamentachse um einen Abstand "a" beabstandet ist, wobei jede Spitze des Filaments auf einem Inkreis liegt, der einen Radius aufweist, der im Wesentlichen einer Länge (a + b) gleich ist,
wobei das Filament ein Modifikationsverhältnis (MV) aufweist, das durch das Verhältnis des Radius (a + b) des Inkreises zum Radius (c) des Inkreises definiert ist, wobei
das Filament ein Denier pro Filament ("pdf") im Bereich von 10<"pdf"<35 aufweist;
der Abstand "a" im Bereich von 0,00025 Zoll (6 Mikrometern) <"a"<0,004 Zoll (102 Mikrometern) liegt;
der Abstand "b" im Bereich von 0,00008 Zoll (2 Mikrometern) <"b"<0,0010 Zoll (24 Mikrometern) liegt;
der Abstand "c" im Bereich von 0,0003 Zoll (8 Mikrometern) <"c"<0,0025 Zoll (64 Mikrometern) liegt; und
das Modifikationsverhältnis ("MV") im Bereich von etwa 1,1<"MV"<etwa 2,0 liegt, wobei das synthetische Polymer Polytrimethylenterephthalat ist.

2. Teppich, der eine Rückenbeschichtung und eine Vielzahl von Noppen aufweist, die an der Rückenbeschichtung befestigt sind,
wobei jede Noppe ein fibrillierungsresistentes, synthetisches polymeres Filament mit festem Kern nach Anspruch 1 aufweist.

3. Filament oder Teppich nach Anspruch 1 oder 2, wobei das Filament eine Zähigkeit von mehr als 1,5 Gramm pro Denier aufweist.

4. Filament oder Teppich nach Anspruch 1 oder 2, wobei
das Filament ein Denier pro Filament ("pdf") im Bereich von 12<"pdf"<32 aufweist;
der Abstand "a" im Bereich von 0,00035 Zoll (9 Mikrometern) <"a"<0,003 Zoll (76 Mikrometern) liegt;
der Abstand "b" im Bereich von 0,00010 Zoll (3 Mikrometern) <"b"<0,00095 Zoll (25 Mikrometern) liegt;
der Abstand "c" im Bereich von 0,0005 Zoll (10 Mikrometern) <"c"<0,002 Zoll (51 Mikrometern) liegt; und
das Modifikationsverhältnis ("MV") im Bereich von etwa 1,1 <"MV"<etwa 2,0 liegt.

5. Filament oder Teppich nach Anspruch 1, wobei das Polytrimethylenterephthalat ein Mattierungsmittel darin aufweist.

6. Filament oder Teppich nach Anspruch 1, wobei das Polytrimethylenterephthalat pigmentiert ist.

7. Filament oder Teppich nach Anspruch 1, wobei das Polytrimethylenterephthalat ein 1,3-Propandiol aufweist, das biologisch hergestellt worden ist.

8. Filament oder Teppich nach Anspruch 1, wobei das Polytrimethylenterephthalat ein Flammhemmungsmittel darin aufweist.

9. Spinndüsenplatte zum Bilden eines fibrillierungsresistenten, synthetischen, polymeren Filaments mit festem Kern, das eine Längsachse, die sich darin hindurch erstreckt, und einen dreiseitigen Querschnitt in einer zur Längsachse senkrechten Ebene aufweist,
wobei die Spinndüsenplatte eine Vielzahl von Öffnungen, die darin gebildet sind, aufweist, wobei jede Öffnung eine Mitte und frei Seiten aufweist, wobei jede Seite an einem ersten und einem zweiten Endpunkt endet, wobei jede Seite einen Mittelpunkt zwischen dem ersten und dem zweiten Endpunkt aufweist,
wobei der erste Endpunkt einer Seite mit dem zweiten Endpunkt einer benachbarten Seite durch eine kreisförmige Endkontur verbunden ist, wobei die kreisförmige Endkontur einen Radius aufweist, der einer Dimension "C" gleich ist, die von einem mittleren Punkt aus gemessen wird, der auf einer von der Mitte der Öffnung ausgehenden Radiallinie liegt, wobei der mittlere Punkt jeder Endkontur sich in einem vorbestimmten Abstand "D" von der Mitte der Öffnung befindet,
wobei der erste Endpunkt jeder Seite von dem zweiten Endpunkt einer benachbarten Seite einer Sehne entlang, die zwischen den Endpunkten benachbarter Seiten definiert ist, beabstandet ist, und
ein Punkt auf jeder kreisförmigen Endkontur auf einem Inkreis liegt, der einen Radius ("C+D") aufweist, der auf die Mitte der Öffnung zentriert ist, wobei die Mittelpunkte jeder Seite auf einem Inkreis liegen, der einen Radius "H" aufweist, der auf den mittleren Punkt der Öffnung zentriert ist,
wobei
der Abstand "C" im Bereich von 0,0015 Zoll (38 Mikrometern) <"C"<0,0040 Zoll (102 Mikrometern) liegt;
der Abstand "D" im Bereich von 0,0150 Zoll (381 Mikrometern) <"D"<0,0300 Zoll (762 Mikrometern) liegt.

10. Spinndüsenplatte nach Anspruch 9, wobei
der Abstand "C" im Bereich von 0,0020 Zoll (51 Mikrometern) <"C"<0,0035 Zoll (89 Mikrometern) liegt;
der Abstand "D" im Bereich von 0,0175 Zoll (445 Mikrometern) <"D"<0,0280 Zoll (711 Mikrometern) liegt.

11. Spinndüsenplatte nach Anspruch 9, wobei jeder Endpunkt jeder Seite ein Berührungspunkt einer kreisförmigen Endkontur ist.

12. Spinndüsenplatte nach Anspruch 9, wobei
jede Seite jeder Öffnung im Wesentlichen konkav ist, wobei jede Seite auf einem Bezugskreis liegt, der eine Mitte aufweist, die auf einem Bezugsradius gelegen ist, der aus dem mittleren Punkt der Öffnung ausgeht und durch einen Mittelpunkt einer Seite hindurchgeht,
wobei die Mitte des Bezugskreises sich in einem vorbestimmten Abstand "A" dem Bezugsradius von der Mittelachse der Öffnung entlang befindet, wobei der Bezugskreis einen Dimensionsradius "B" aufweist,
die Öffnung ein Modifikationsverhältnis ("MV") aufweist, das durch das Verhältnis des Radius (C+D) des Inkreises zum Radius (A-B) des Inkreises definiert ist, sodass $ʺMVʺ = \left(C+D\right) / ʺHʺ ,$
wenn
der Abstand "A" im Bereich von 0,0300 Zoll (762 Mikrometern) <"A"<0,0900 Zoll (2286 Mikrometern) liegt;
der Abstand "B" im Bereich von 0,0200 Zoll (508 Mikrometern) <"B"<0,0800 Zoll (2032 Mikrometern) liegt;
das Verhältnis (A/B) innerhalb des Bereichs von etwa 1,0 <(A/B)<etwa 1,6 liegt; und
das Modifikationsverhältnis ("MV") im Bereich von etwa 1,5 <"MV"<etwa 4,5 liegt.

13. Spinndüsenplatte nach Anspruch 12, wobei
der Abstand "A" im Bereich von 0,0300 Zoll (762 Mikrometern) <"A"<0,0800 Zoll (2032 Mikrometern) liegt;
der Abstand "B" im Bereich von 0,0200 Zoll (508 Mikrometern) <"B"<0,0700 Zoll (1778 Mikrometern) liegt;
das Verhältnis (A/B) innerhalb des Bereichs von etwa 1,1 <(A/B)<etwa 1,5 liegt; und
das Modifikationsverhältnis ("MV") im Bereich von etwa 1,8 <"MV"<etwa 3,5 liegt.

14. Spinndüsenplatte nach Anspruch 9, wobei jede Seite jeder Öffnung im Wesentlichen linear ist,
wobei ein Punkt auf jeder kreisförmigen Endkontur auf einem Inkreis liegt, der einen Radius "(C+D)" aufweist, der auf die Mitte der Öffnung zentriert ist,
wobei Mittelpunkte jeder Seite auf einem Inkreis liegen, der einen Radius "H" aufweist, der auf die Mitte der Öffnung zentriert ist, wobei
der Abstand "H im Bereich von 0,0090 Zoll (229 Mikrometern) <"H"<0,0190 Zoll (483 Mikrometern) liegt;
wobei die Öffnung ein Modifikationsverhältnis ("MV") aufweist, das durch das Verhältnis des Radius (C+D) des Inkreises zum Radius "H" des Inkreises definiert ist, sodass $ʺMVʺ = \left(C+D\right) / ʺHʺ ,$
wobei
das Modifikationsverhältnis ("MV") im Bereich von etwa 1,6<"MV"<etwa 2,5 liegt.

15. Spinndüsenplatte nach Anspruch 14, wobei
der Abstand "H (d.h. der Radius der Inkreises) im Bereich von 0,0108 Zoll (274 Mikrometern) <"H"<0,0175 Zoll (445 Mikrometern) liegt;
das Modifikationsverhältnis ("MV") im Bereich von etwa 1,7 <"MV"<etwa 2,3 liegt.

16. Spinndüsenplatte zum Bilden eines fibrillierungsresistentes, synthetischen, polymeren Filaments mit festem Kern, das eine Längsachse, die sich darin hindurch erstreckt, und einen dreiseitigen Querschnitt in einer zur Längsachse senkrechten Ebene aufweist,
wobei die Spinndüsenplatte eine Vielzahl von Öffnungen, die darin gebildet sind, aufweist, wobei jede Öffnung eine Mitte und drei Seiten aufweist, wobei jede Seite in einem ersten und einem zweiten Endpunkt endet, wobei jede Seite einen Mittelpunkt zwischen dem ersten und dem zweiten Endpunkt aufweist,
wobei der erste Endpunkt jeder Seite von dem zweiten Endpunkt einer benachbarten Seite durch eine Basislinie beabstandet ist, die zwischen den Endpunkten benachbarter Seiten definiert ist, wobei die Basislinie einen Bezugsradius überschneidet, der aus dem mittleren Punkt ausgeht, wobei der Schnittpunkt zwischen der Basislinie und dem Bezugsradius in einem Abstand "G" dem Bezugsradius entlang von der Mitte der Öffnung aus liegt, wobei die Basislinie eine vorbestimmte Länge "2F" aufweist,
wobei der erste Endpunkt einer Seite mit dem zweiten Endpunkt einer benachbarten Seite durch eine Endkontur verbunden ist, die mindestens zwei lineare Kanten aufweist, wobei die linearen Kanten sich in einem Gipfel überschneiden, wobei der Gipfel von der Schnittstelle der Basislinie und des Bezugsradius durch eine Dimension "E" beabstandet ist, wobei
der Abstand "E" im Bereich von 0,0025 Zoll (64 Mikrometern) <"E"<0,0150 Zoll (381 Mikrometern) liegt;
der Abstand "F" im Bereich von 0,015 Zoll (38 Mikrometern) <"F"<0,0040 Zoll (102 Mikrometern) liegt.
der Abstand "G" im Bereich von 0,0150 Zoll (381 Mikrometern) <"G"<0,0300 Zoll (762 Mikrometern) liegt.

17. Spinndüsenplatte nach Anspruch 16, wobei
der Abstand "E" im Bereich von 0,0030 Zoll (76 Mikrometern) <"E"<0,0100 Zoll (254 Mikrometern) liegt;
der Abstand "F" im Bereich von 0,0020 Zoll (51 Mikrometern) <"F"<0,0035 Zoll (89 Mikrometern) liegt und
der Abstand "G" im Bereich von 0,0175 Zoll (445 Mikrometern) <"G"<0,0280 Zoll (711 Mikrometern) liegt.

18. Spinndüsenplatte nach Anspruch 16, wobei
jede Seite jeder Öffnung im Wesentlichen konkav ist, wobei jede Seite auf einem Bezugskreis liegt, der eine Mitte aufweist, die auf einem Bezugsradius gelegen ist, der aus dem mittleren Punkt der Öffnung ausgeht und durch einen Mittelpunkt einer Seite hindurchgeht,
wobei die Mitte des Bezugskreises sich in einem vorbestimmten Abstand "A" dem Bezugsradius von der Mittelachse der Öffnung entlang befindet, wobei der Bezugskreis einen Dimensionsradius "B" aufweist,
die Öffnung ein Modifikationsverhältnis ("MV") aufweist, das durch das Verhältnis des Radius (E+G) des Inkreises zum Radius "(E+G)" des Inkreises definiert ist, sodass $ʺMVʺ = \left(C+D\right) / \left(A-B\right) ⁢ ʺ ,$
wobei
der Abstand "A" im Bereich von 0,0300 Zoll (762 Mikrometern) <"A"<0,0900 Zoll (2286 Mikrometern) liegt;
der Abstand "B" im Bereich von 0,0200 Zoll (508 Mikrometern) <"B"<0,0800 Zoll (2032 Mikrometern) liegt;
das Verhältnis (A/B) innerhalb des Bereichs von etwa 1,0 <(A/B)<etwa 1,6 liegt; und
das Modifikationsverhältnis ("MV") im Bereich von etwa 1,5 <"MV"<etwa 4,5 liegt.

19. Spinndüsenplatte nach Anspruch 18, wobei
der Abstand "A" im Bereich von 0,0300 Zoll (762 Mikrometern) <"A"<0,0800 Zoll (2032 Mikrometern) liegt;
der Abstand "B" im Bereich von 0,0200 Zoll (508 Mikrometern) <"B"<0,0800 Zoll (1778 Mikrometern) liegt;
das Verhältnis (A/B) innerhalb des Bereichs von etwa 1,1 <(A/B)<etwa 1,5 liegt; und
das Modifikationsverhältnis ("MV") im Bereich von etwa 1,8 <"MV"<etwa 3,5 liegt.

20. Spinndüsenplatte nach Anspruch 18, wobei jede Seite jeder Öffnung im Wesentlichen linear ist,
wobei der Gipfel auf jeder kreisförmigen Endkontur auf einem Inkreis liegt, der einen Radius ("G+E") aufweist, der auf die Mitte der Öffnung zentriert ist,
wobei die Mittelpunkte jeder Seite auf einem Inkreis liegen, der einen Radius "H" aufweist, der auf die Mitte der Öffnung zentriert ist, wobei
der Abstand "H im Bereich von 0,0088 Zoll (224 Mikrometern) <"H"<0,0185 Zoll (470 Mikrometern) liegt;
wobei die Öffnung ein Modifikationsverhältnis ("MV") aufweist, das durch das Verhältnis des Radius (G+E) des Inkreises zum Radius "H" des Inkreises definiert ist, sodass $ʺMVʺ = \left(G+E\right) / ʺ ⁢ H ⁢ ʺ ,$
wobei
das Modifikationsverhältnis ("MV") im Bereich von etwa 1,6 <"MV"<etwa 2,5 liegt.

21. Spinndüsenplatte nach Anspruch 20, wobei
der Abstand "H (d.h. der Radius der Inkreises) im Bereich von 0,0105 Zoll (267 Mikrometern) <"H"<0,0170 Zoll (432 Mikrometern) liegt;
das Modifikationsverhältnis ("MV") im Bereich von etwa 1,7 <"MV"<etwa 2,3 liegt.

22. Verfahren zur Herstellung eines fibrillierungsresistenten, synthetischen, polymeren Filaments mit festem Kern, das eine Längsachse, die sich darin hindurch erstreckt, und einen dreiseitigen Querschnitt in einer zur Längsachse senkrechten Ebene aufweist,
wobei die Seiten im Wesentlichen längenmäßig gleich sind und eine konvexe Form aufweisen, wobei jede Seite einen Mittelpunkt daran entlang aufweist, wobei jeder Mittelpunkt auf einem Inkreis liegt, der auf die Mittelachse des Filaments zentriert ist, wobei der Inkreis einen Radius aufweist, der einer Länge "c" im Wesentlichen gleich ist,
wobei jede Seite auf eine benachbarte Seite durch eine im Wesentlichen abgerundete Spitze auftrifft, die auf einen entsprechenden Krümmungskreis zentriert ist, wobei jeder Krümmungskreis einen Radius aufweist, der einer Länge "b" im Wesentlichen gleich ist, wobei jeder Krümmungskreis von der Filamentachse um einen Abstand "a" beabstandet ist, wobei jede Spitze des Filaments auf einem Inkreis liegt, der einen Radius aufweist, der im Wesentlichen einer Länge (a + b) gleich ist,
wobei das Filament ein Modifikationsverhältnis (MV) aufweist, das durch das Verhältnis des Radius (a + b) des Inkreises zum Radius (c) des Inkreises definiert ist, wobei
das Filament ein Denier pro Filament ("pdf") im Bereich von 10<"pdP'<35 aufweist;
der Abstand "a" im Bereich von 0,00025 Zoll (6 Mikrometern) <"a"<0,004 Zoll (102 Mikrometern) liegt;
der Abstand "b" im Bereich von 0,00008 Zoll (2 Mikrometern) <"b"<0,0010 Zoll (24 Mikrometern) liegt;
der Abstand "c" im Bereich von 0,0003 Zoll (8 Mikrometern) <"c"<0,0025 Zoll (64 Mikrometern) liegt; und
das Modifikationsverhältnis ("MV") im Bereich von etwa 1,1 <"MV"<etwa 2,0 liegt,
wobei das Verfahren die Schritte umfasst des:
a) Pumpens von geschmolzenem synthetischem Polymer durch die Spinndüsenplatte nach Anspruch 11 und/oder Anspruch 18, die eine Vielzahl von Öffnungen aufweist, unter Bildung von Filamenten, wobei das synthetische Polymer Polytrimethylenterephthalat ist;
b) Kühlens der Filamente;
c) Aufbringens einer Appretur auf die Filamente;
d) Streckens und Temperns der Filamente; und
d) Aufbauschens der Filamente, um den Filamenten eine willkürliche, dreidimensionale, gekrümmte Kräuselung zu verleihen.

23. Verfahren nach Anspruch 22, wobei
wobei jede Öffnung der Spinndüsenplatte eine Mitte und drei Seiten aufweist, wobei jede Seite an einem ersten und einem zweiten Endpunkt endet, wobei jede Seite einen Mittelpunkt zwischen dem ersten und dem zweiten Endpunkt aufweist,
wobei der erste Endpunkt einer Seite mit dem zweiten Endpunkt einer benachbarten Seite durch eine kreisförmige Endkontur verbunden ist, wobei die kreisförmige Endkontur einen Radius aufweist, der einer Dimension "C" gleich ist, die von einem mittleren Punkt aus gemessen wird, der auf einer von der Mitte der Öffnung ausgehenden Radiallinie liegt, wobei der mittlere Punkt jeder Endkontur sich in einem vorbestimmten Abstand "D" von der Mitte der Öffnung befindet,
wobei der erste Endpunkt jeder Seite von dem zweiten Endpunkt einer benachbarten Seite einer Sehne entlang, die zwischen den Endpunkten der benachbarten Seiten definiert ist, beabstandet ist, und
ein Punkt auf jeder kreisförmigen Endkontur auf einem Inkreis liegt, der einen Radius "(C+D)" aufweist, der auf die Mitte der Öffnung zentriert ist, wobei die Mittelpunkte jeder Seite auf einem Inkreis liegen, der einen Radius "H" aufweist, der auf die Mitte der Öffnung zentriert ist,
wobei
der Abstand "C" im Bereich von 0,0015 Zoll (38 Mikrometern) <"C"<0,0040 Zoll (102 Mikrometern) liegt.
der Abstand "D" im Bereich von 0,0150 Zoll (381 Mikrometern) <"D"<0,0300 Zoll (762 Mikrometern) liegt.

24. Verfahren nach Anspruch 22, wobei
wobei jede Öffnung der Spinndüsenplatte eine Mitte und drei Seiten aufweist, wobei jede Seite an einem ersten und einem zweiten Endpunkt endet, wobei jede Seite einen Mittelpunkt zwischen dem ersten und dem zweiten Endpunkt aufweist,
wobei der erste Endpunkt jeder Seite von dem zweiten Endpunkt einer benachbarten Seite durch eine Basislinie beabstandet ist, die zwischen den Endpunkten benachbarter Seiten definiert ist, wobei die Basislinie einen Bezugsradius überschneidet, der aus dem mittleren Punkt ausgeht, wobei der Schnittpunkt zwischen der Basislinie und dem Bezugsradius in einem Abstand "G" dem Bezugsradius entlang von der Mitte der Öffnung aus liegt, wobei die Basislinie eine vorbestimmte Länge "2F" aufweist,
wobei der erste Endpunkt einer Seite mit dem zweiten Endpunkt einer benachbarten Seite durch eine Endkontur verbunden ist, die mindestens zwei lineare Kanten aufweist, wobei die linearen Kanten sich in einem Gipfel überschneiden, wobei der Gipfel von der Schnittstelle der Basislinie und des Bezugsradius durch eine Dimension "E" beabstandet ist, wobei
der Abstand "E" im Bereich von 0,0025 Zoll (64 Mikrometern) <"E"<0,150 Zoll (381 Mikrometern) liegt;
der Abstand "F" im Bereich von 0,015 Zoll (38 Mikrometern) <"F"<0,0040 Zoll (102 Mikrometern) liegt.
der Abstand "G" im Bereich von 0,0150 Zoll (381 Mikrometern) <"G"<0,0300 Zoll (762 Mikrometern) liegt.

25. Verfahren nach Anspruch 22, wobei das Polytrimethylenterephthalat ein 1,3-Propandiol aufweist, das biologisch hergestellt worden ist.

## Revendications

1. Filament polymère synthétique, résistant à la fibrillation, à âme pleine ayant un
axe longitudinal se situant à travers et une section transversale triangulaire dans un plan perpendiculaire à l'axe longitudinal,
les faces étant substantiellement égales en longueur et de forme convexe, chaque face ayant un point médian le long de celle-ci, chaque point médian se situant sur un cercle inscrit centré sur l'axe central du filament, le cercle inscrit ayant un rayon substantiellement égal à une longueur « c »,
chaque face rencontrant une face adjacente à travers une extrémité substantiellement arrondie centrée sur un cercle respectif de courbure, chaque cercle de courbure ayant un rayon substantiellement égal à une longueur « b », chaque cercle de courbure étant espacé de l'axe du filament d'une distance « a », chaque extrémité du filament se situant sur un cercle circonscrit ayant un rayon substantiellement égal à une longueur (a+b),
le filament ayant un rapport de modification (RM) définit par le rapport du rayon (a+b) du cercle circonscrit du rayon (c) du cercle inscrit,
dans lequel
le filament a un denier par filament (« dpf ») situé dans la plage de 10<«dpf»<35;
la distance « a » se situe dans la plage de 0,00025 pouce (6 micromètres) < « a » < 0,004 pouce (102 micromètres);
la distance « b » se situe dans la plage de 0,00008 pouce (2 micromètres) < « b » < 0,0010 pouce (24 micromètres);
la distance « c » se situe dans la plage de 0,0003 pouce (8 micromètres) < « c » < 0,0025 pouce (64 micromètres); et
le rapport de modification (« RM ») se situe dans la plage d'environ 1,1 < « RM » < environ 2,0, dans lequel le polymère synthétique est un (poly)téréphtalate de triméthylène.

2. Tapis ayant un envers et une pluralité de touffes fixées à l'envers,
chaque touffe ayant un filament polymère synthétique, résistant à la fibrillation à âme pleine, tel que revendiqué selon la revendication 1.

3. Filament ou tapis selon les revendications 1 ou 2 dans lequel le filament a une ténacité supérieure à 1,5 gramme par denier.

4. Filament ou tapis selon les revendications 1 ou 2 dans lequel
le filament a un denier par filament (« dpf ») dans la plage de 12 < « dpf » < 32;
la distance « a » se situe dans la plage de 0,00035 pouce (9 micromètres) < « a » < 0,003 pouce (76 micromètres);
la distance « b » se situe dans la plage de 0,00010 pouce (3 micromètres) < « b » < 0,00095 pouce (25 micromètres);
la distance « c » se situe dans la plage de 0,0005 pouce (10 micromètres) < « c » < 0,002 pouce (51 micromètres); et
le rapport de modification (« RM ») se situe dans la plage d'environ 1,1 < « RM » < environ 2,0.

5. Filament ou tapis selon la revendication 1 dans lequel le (poly)téréphtalate de triméthylène possède un délustrant à l'intérieur.

6. Filament ou tapis selon la revendication 1 dans lequel le (poly)téréphtalate de triméthylène est pigmenté.

7. Filament ou tapis selon la revendication 1 dans lequel le (poly)téréphtalate de triméthylène a un 1,3 propane diol qui est biologiquement produit.

8. Filament ou tapis selon la revendication 1 dans lequel le (poly)téréphtalate de triméthylène a un agent ignifuge à l'intérieur.

9. Plaque de filières pour la formation d'un filament polymère synthétique, résistant à la fibrillation, à âme pleine ayant un axe longitudinal se situant à travers et une section transversale triangulaire dans un plan perpendiculaire à l'axe longitudinal,
la plaque de filières ayant une pluralité d'orifices formés à l'intérieur, chaque orifice ayant un centre et trois faces, chaque face se terminant en un premier et un second points d'extrémité, chaque face ayant un point médian entre les premier et second points d'extrémité,
le premier point d'extrémité sur une face étant connecté au second point d'extrémité d'une face adjacente grâce à un contour d'extrémité circulaire, le contour d'extrémité circulaire ayant un rayon égal à une dimension « C » mesurée à partir d'un point central se situant sur la ligne radiale émanant du centre de l'orifice, le point central de chaque contour d'extrémité étant disposé à une distance prédéterminée « D » à partir du centre de l'orifice,
le premier point d'extrémité de chaque face étant espacé du second point d'extrémité d'une face adjacente le long d'une corde définie entre les points d'extrémités des faces adjacentes, et,
un point sur chaque contour d'extrémité circulaire se situant sur un cercle circonscrit ayant un rayon « (C+D) » centré sur le centre de l'orifice, les points médians de chaque face se situant sur un cercle inscrit ayant un rayon « H » centré sur le centre de l'orifice,
dans lequel
la distance « C » se situe dans la plage de 0,0015 pouce (38 micromètres) < « C » < 0,0040 pouce (102 micromètres);
la distance « D » se situe dans la plage de 0,0150 pouce (381 micromètres) < « D » < 0,0300 pouce (762 micromètres).

10. Plaque de filières selon la revendication 9 dans laquelle
la distance « C » se situe dans la plage de 0,0020 pouce (51 micromètres) < « C » < 0,0035 pouce (89 micromètres);
la distance « D » se situe dans la plage de 0,0175 pouce (445 micromètres) < « D » < 0,0280 pouce (711 micromètres).

11. Plaque de filières selon la revendication 9 dans laquelle chaque point d'extrémité de chaque face est un point de tangence d'un contour d'extrémité circulaire.

12. Plaque de filières selon la revendication 9 dans laquelle
chaque face de chaque orifice est substantiellement concave avec chaque face se situant sur un cercle de référence ayant un centre localisé sur un rayon de référence émanant du point central de l'orifice et passant à travers un point médian d'une face,
le centre du cercle de référence étant disposé à une distance prédéterminée « A » le long du rayon de référence à partir de l'axe central de l'orifice, le cercle de référence ayant un rayon d'une dimension « B »,
l'orifice a un rapport de modification (« RM ») défini par le rapport du rayon (C+D) du cercle circonscrit au rayon « (A-B) » du cercle inscrit, ainsi, $«RM» = \left(C+D\right) / «H» ,$
dans laquelle
la distance « A » se situe dans la plage de 0,0300 pouce (762 micromètres) < « A » < 0,0900 pouce (2 286 micromètres);
la distance « B » se situe dans la plage de 0,0200 pouce (508 micromètres) < « B » < 0,0800 pouce (2 032 micromètres);
le ratio (A/B) se situe dans la plage d'environ 1,0 < (A/B) < environ 1,6; et
le rapport de modification (« RM ») se situe dans la plage d'environ 1,5 < « RM » < à environ 4,5.

13. Plaque de filières selon la revendication 12 dans laquelle
la distance « A » se situe dans la plage de 0,0300 pouce (762 micromètres) < « A » < 0,0800 pouce (2 032 micromètres);
la distance « B » se situe dans la plage de 0,0200 pouce (508 micromètres) < « B » < 0,0700 pouce (1 778 micromètres);
le rapport (A/B) se situe dans la plage d'environ 1,1 < (A/B) < environ 1,5; et
le rapport de modification (« RM ») se situe dans la plage d'environ 1,8 < « RM » < environ 3,5.

14. Plaque de filières selon la revendication 9 dans laquelle chaque face de chaque orifice est substantiellement linéaire,
un point de chaque contour d'extrémité circulaire se situant sur un cercle circonscrit ayant un rayon « (C+D) » centré sur le centre de l'orifice,
les points médians de chaque face se situant sur un cercle inscrit ayant un rayon « H » centré sur le centre de l'orifice, dans laquelle
la distance « H » se situe dans la plage de 0,0090 pouce (229 micromètres) < « H » < 0,0190 pouce (483 micromètres),
l'orifice a un rapport de modification (« RM ») défini par le rapport du rayon (C+D) du cercle circonscrit au rayon « H » du cercle inscrit, ainsi, $«RM» = \left(C+D\right) / «H» ,$
dans lequel
le rapport de modification (« RM ») se situe dans la plage d'environ 1,6 < « RM » < environ 2,5.

15. Plaque de filières selon la revendication 14 dans laquelle
la distance « H » (c'est-à-dire, le rayon du cercle inscrit) se situe dans la plage allant de 0,0108 pouce (274 micromètres) < « H » < 0,0175 pouce (445 micromètres)
le rapport de modification (« RM ») se situe dans la plage d'environ 1,7 < « RM » < environ 2,3.

16. Plaque de filières pour former un filament polymère synthétique résistant à la fibrillation à âme pleine ayant un axe longitudinal se situant à travers et une section transversale triangulaire dans un plan perpendiculaire à l'axe longitudinal,
la plaque de filières ayant une pluralité d'orifices formés à l'intérieur, chaque orifice ayant un centre et trois faces, chaque face se terminant en un premier et un second points d'extrémité, chaque face ayant un point médian entre les premier et second points d'extrémité,
le premier point d'extrémité de chaque face étant espacé du second point d'extrémité d'une face adjacente d'une ligne de référence définie entre les points d'extrémité des faces adjacentes, la ligne de référence entrant en intersection avec un rayon de référence émanant du point central, le point d'intersection entre la ligne de référence et le rayon de référence se situant d'une distance « G » le long du rayon de référence à partir du centre de l'orifice, la ligne de référence ayant une longueur prédéterminée « 2F »,
le premier point d'extrémité d'une face étant connecté au second point d'extrémité d'une face adjacente par un contour d'extrémité ayant au moins deux bords linéaires, les bords linéaires entrant en intersection dans un apex, l'apex étant espacé de l'intersection de la ligne de référence et du rayon de référence d'une dimension « E », dans laquelle
la distance « E » se situe dans la plage de 0,0025 pouce (64 micromètres) < « E » < 0,0150 pouce (381 micromètres);
la distance « F » se situe dans la plage de 0,0015 pouce (38 micromètres) < « F » < 0,0040 pouce (102 micromètres); et
la distance « G » se situe dans la plage de 0,0150 pouce (381 micromètres) < « G » < 0,0300 pouce (762 micromètres).

17. Plaque de filières selon la revendication 16 dans laquelle
la distance « E » se situe dans la plage de 0,0030 pouce (76 micromètres) < « E » < 0,0100 pouce (254 micromètres);
la distance « F » se situe dans la plage de 0,0020 pouce (51 micromètres) < « F » < 0,0035 pouce (89 micromètres); et
la distance « G » se situe dans la plage de 0,0175 pouce (445 micromètres) < « G » < 0,0280 pouce (711 micromètres).

18. Plaque de filières selon la revendication 16 dans laquelle
chaque face de chaque orifice est substantiellement concave avec chaque face se situant sur un cercle de référence ayant un centre localisé sur un rayon de référence émanant du point central de l'orifice et passant à travers un point médian d'une face,
le centre du cercle de référence étant disposé à une distance prédéterminée « A » le long du rayon de référence depuis l'axe central de l'orifice, le cercle de référence ayant un rayon de dimension « B »,
l'orifice a un rapport de modification (« RM ») défini par le rapport du rayon (E+G) du cercle circonscrit au rayon « (E+G) » du cercle inscrit, ainsi, $«RM» = \left(C+D\right) / « ⁢ \left(A-B\right) ⁢ » ,$
dans laquelle la distance « A » se situe dans la plage de 0,0300 pouce (762 micromètres) < « A » < 0,0900 pouce (2 286 micromètres);
la distance « B » se situe dans la plage de 0,0200 pouce (508 micromètres) < « B » < 0,0800 pouce (2 032 micromètres);
le rapport (A/B) se situe dans la plage d'environ 1,0 < (A/B) < environ 1,6; et
le rapport de modification (« RM ») se situe dans la plage d'environ 1,5 < « RM » < environ 4,5.

19. Plaque de filières selon la revendication 18 dans laquelle
la distance « A » se situe dans la plage de 0,0300 pouce (762 micromètres) < « A » < 0,0800 pouce (2 032 micromètres);
la distance « B » se situe dans la plage de 0,0200 pouce (508 micromètres) < « B » < 0,0800 pouce (1 778 micromètres);
le rapport (A/B) se situe dans la plage d'environ 1,1 < (A/B) < environ 1,5; et
le rapport de modification (« RM ») se situe dans la plage d'environ 1,8 < « RM » < environ 3,5.

20. Plaque de filières selon la revendication 16 dans laquelle chaque face de chaque orifice est substantiellement linéaire,
l'apex sur chaque contour d'extrémité circulaire se situant sur un cercle circonscrit ayant un rayon « (G+E) » centré sur le centre de l'orifice,
les points médians de chaque face se situant sur un cercle inscrit ayant un rayon « H » centré sur le centre de l'orifice, dans lequel
la distance « H » se situe dans la plage de 0,0088 pouce (224 micromètres) < « H » < 0,0185 pouce (470 micromètres),
l'orifice a un rapport de modification (« RM ») défini par le rapport du rayon (G+E) du cercle circonscrit au rayon « H » du cercle inscrit, ainsi, $«RM» = \left(G+E\right) / «H» ,$
dans laquelle
le rapport de modification (« RM ») se situe dans la plage d'environ 1,6 < « RM » < environ 2,5.

21. Plaque de filières selon la revendication 20 dans laquelle
la distance « H » (c'est-à-dire, le rayon du cercle inscrit) se situe dans la plage de 0,0105 pouce (267 micromètres) < « H » < 0,0170 pouce (432 micromètres)
le rapport de modification (« RM ») se situe dans la plage d'environ 1,7 < « RM » < environ 2,3.

22. Procédé de fabrication d'un filament polymère synthétique, résistant à la fibrillation, à âme pleine ayant un axe longitudinal se situant à travers et une section transversale triangulaire dans un plan perpendiculaire à l'axe longitudinal,
les faces étant substantiellement égales de longueur et convexe de forme, chaque face ayant un point médian dans sa longueur, chaque point médian se situant sur un cercle inscrit centré sur l'axe central du filament, le cercle inscrit ayant un rayon substantiellement égal à une longueur « c »,
chaque face rencontrant une face adjacente à travers une extrémité substantiellement arrondie centrée sur un cercle respectif de courbure, chaque cercle de courbure ayant un rayon substantiellement égal à une longueur « b », chaque cercle de courbure étant espacé de l'axe du filament d'une distance « a », chaque extrémité du filament se situant sur un cercle circonscrit ayant un rayon substantiellement égal à une longueur (a+b),
le filament ayant un rapport de modification (RM) défini par le rapport du rayon (a+b) du cercle circonscrit au rayon (c) du cercle inscrit, dans lequel
le filament a un denier par filament (« dpf ») dans la plage de 10 < « dpf » < 35;
la distance « a » se situe dans la plage de 0,00025 pouce (6 micromètres) < « a » < 0,004 pouce (102 micromètres);
la distance « b » se situe dans la plage de 0,00008 pouce (2 micromètres) < « b » < 0,0010 pouce (24 micromètres);
la distance « c » se situe dans la plage de 0,0003 pouce (8 micromètres) < « c » < 0,0025 pouce (64 micromètres); et
le rapport de modification (« RM ») se situe dans la plage d'environ 1,1 < « RM » < environ 2,0,
le procédé comprend les étapes de:
a) pompage du polymère synthétique fondu à travers ladite plaque de filières selon la revendication 11 et/ou selon la revendication 18 ayant une pluralité d'orifices pour former des filaments dans lequel le polymère synthétique est du (poly)téréphtalate de triméthylène;
b) refroidissement des filaments;
c) application d'un fini aux filaments;
d) étirage et hybridation des filaments; et
e) étoffement des filaments pour conférer une frisure curvilinéaire tridimensionnelle aléatoire aux filaments.

23. Procédé selon la revendication 22 dans lequel
chaque orifice de la plaque de filières a un centre et trois faces, chaque face se terminant en un premier et un second points de terminaison, chaque face ayant un point médian entre les premier et second points de terminaison,
le premier point de terminaison d'une face étant connecté au second point de terminaison d'une face adjacente d'un contour d'extrémité circulaire, le contour d'extrémité circulaire ayant un rayon égal à une dimension « C » mesurée à partir d'un point central se situant sur une ligne radiale émanant du centre de l'orifice, le point central de chaque contour d'extrémité étant disposé selon une distance prédéterminée « D » à partir du centre de l'orifice,
le premier point d'extrémité de chaque face étant espacé du second point d'extrémité d'une face adjacente le long d'une corde définie entre les points d'extrémité des faces adjacentes, et,
un point sur chaque contour d'extrémité circulaire se situant sur un cercle circonscrit ayant un rayon « (C+D) » centré sur le centre de l'orifice, les points médians de chaque face se situant sur un cercle inscrit ayant un rayon « H » centré sur le centre de l'orifice,
dans lequel
la distance « C » se situe dans la plage de 0,0015 pouce (38 micromètres) < « C » < 0,0040 pouce (102 micromètres);
la distance « D » se situe dans la plage de 0,0150 pouce (381 micromètres) < « D » < 0,0300 pouce 762 micromètres).

24. Procédé selon la revendication 22 dans lequel
chaque orifice de la plaque de filières a un centre et trois faces, chaque face se terminant en un premier et un second points d'extrémité, chaque face ayant un point médian entre les premier et second points d'extrémité,
le premier point d'extrémité de chaque face étant espacé du second point d'extrémité d'une face adjacente par une ligne de référence définie entre les points d'extrémité des faces adjacentes, la ligne de référence entrant en intersection avec un rayon de référence émanant du point central, le point d'intersection entre la ligne de référence et le rayon de référence se situant d'une distance « G » le long du rayon de référence depuis le centre de l'orifice, la ligne de référence ayant une longueur prédéterminée « 2F »,
le premier point d'extrémité d'une face étant connecté au second point d'extrémité d'une face adjacente par un contour d'extrémité ayant au moins deux bords linéaires, les bords linéaires entrant en intersection dans un apex, l'apex étant espacé de l'intersection de la ligne de référence et du rayon de référence d'une dimension « E », dans lequel
la distance « E » se situe dans la plage de 0,0025 pouce (64 micromètres) < « E » < 0,0150 pouce (381 micromètres);
la distance « F » se situe dans la plage de 0,0015 pouce (38 micromètres) < « F » < 0,0040 pouce (102 micromètres); et
la distance « G » se situe dans la plage de 0,0150 pouce (381 micromètres) < « G » < 0,0300 pouce (762 micromètres).

25. Procédé selon la revendication 22 dans lequel le (poly)téréphtalate de triméthylène a un 1,3 propane diol qui est biologiquement produit.
